

## UNITED STATES PATENT OFFICE

1,970,271

## PROCESS OF TANNING HIDES

Max Bergmann, Dresden, Germany

No Drawing. Application July 28, 1933, Serial  
No. 682,632. In Germany August 1, 1932

7 Claims. (Cl. 149—5)

The present invention relates to a process of tanning or dressing hides by means of iron containing tanning materials, and the main feature of this new process consists in that the hides, after having been prepared in the ordinary manner, are treated first with a tanning agent containing iron in combined form and obtained by the treatment of albuminoid substances in the presence of iron salts with acids and substances exercising 5 oxidizing properties, or with oxidizing acids, whereupon the iron-tanned leather thus obtained is further dressed with the aid of another mineral tanning material, such as chrome-, aluminium- and the like tanning material. The albuminoid substances employed for the production of the 10 tanning agent used for the first phase of this combined tanning process have partly been hydrolyzed, but they have also been changed in other respects by the oxidizers, thus forming with 15 the iron a combination which exercises the tanning effect aimed at in this instance.

By treating the hides with the ferro-albuminoid tanning agents a leather is obtained which is characterized by an excellent grain and good 20 filling, thus differing advantageously also from the ordinary iron-tanned leather. By subsequently treating the leather thus obtained with mineral tanning agents, a filling and a body or state of the leather are secured which are quite 25 exceptional with mineral leathers of any other description. It is a surprising fact, that in spite of this excellent filling also the condition of the so-called fattening folds is a very favourable 30 one, and even the inferior or depending parts of the hide present in this leather a very favourable 35 appearance, such as has been impossible to obtain with the aid of the combined tanning processes known so far. The special advantages of the leather thus obtained render it possible to 40 employ it for uppers, as well as for soles and other purposes. The leather is distinguished by a light, uniform colour, for which reason it is also highly suitable for producing coloured 45 leather.

The possibility of subsequently tanning and filling the leather, which has previously been tanned with a ferruginous tanning agent, with copious quantities of other mineral tanning agents is given by the fact, that as ferruginous 50 tanning agent one of such nature is employed which contains albuminoid substances or albuminoid waste products in complex combination. It is by this fact that the leather tanned therewith obtains the property, in spite of having already 55 been tanned through, of absorbing further con-

siderable quantities of other mineral tanning agents ensuring in this way the effect indicated above. For this reason it is important, that the treatment of the leather with chrome tanning agents or the like is effected only after previous 60 treatment with the ferruginous albuminoid tanning agents and not vice versa.

All mineral tanning agents are to be considered for the subsequent additional tanning process, e. g. the customary chrome tanning agents. 65

*Examples of performance*

(1) For the purpose of tanning 500 kilos of true skins or depilated hides, which have previously been slackened, unlimed and, if necessary, 70 bated and pickled, an albuminoid tanning solution is prepared containing about 3% of  $Fe_2O_3$  reckoned on the weight of the employed true skins. An advantageous way for obtaining this ferruginous albuminoid tanning agent consists 75 in heating 50 kilos of chrome shavings or other leather or skin waste, which may also be replaced by the corresponding quantity of parings of skins or scraps of hide or any other albuminoid product, together with an iron salt obtained from 10 80 kilos of scrap iron, e. g. ferric chloride, and with 100 kilos of nitric acid of 22° Bé., during some time to 80—90° C. until total solution has taken place. After cooling this tanning solution is neutralized with a 10% sodium carbonate solution to such an extent that its pH-value equals 85 about 2.

With the aid of this solution which may, if necessary, yet be diluted, the tanning of the true skins is now effected in the vat or suspension 90 tub in the usual manner until the skins are properly bitten through or, in other words, fully permeated by the tanning solution. The skins then are further tanned through while further quantities of sodium carbonate are added until 95 the tanning solution has attained a pH-value of about 4 and the separation of iron in a flocculent state yet remains just avoided, which will be the case after 6 to 8 hours, if the tanning process takes place in the vat. 100

After the skins thus treated have been beaten over the jack for some time, they are tanned a second time with chrome compounds. For this purpose they are suitably fulled for 1 to 2 hours in a chrome-alum solution, containing 2 to 3% 105 of  $Cr_2O_3$  related to the weight of the true skins employed and having a basicity of about  $\frac{1}{2}$ . The skins then are stored for 1 to 2 days and hereafter neutralized with 5% of sodium bicarbonate. They are subsequently washed, greased and dressed in 110

accordance with known methods. Borax, as well as water-glass, may also be used as neutralizing agents, the water-glass imparting to the leather a particularly attractive light colour.

- 5 The described process may also be altered in such a way that the leather, treated with the ferruginous albuminoid tanning agent is neutralized first and subsequently tanned with a strongly basic chrome liquor.
- 10 (2) For the preparation of the tanning solution to be used in the first stage of the tanning process, 50 kilos of shavings or the corresponding quantity of scraps of hide, glue or the like are heated with 50 kilos of iron chloride and 150 liters of 18% hydrochloric acid to about 80 to 90° C. until the mass will be fully dissolved. In order to oxidize the iron salt, for instance 20 kilos of potassium chloride then are gradually added to the solution, which is further heated until the reaction is completed. This will be the case when the frothing has ceased. The solution thus obtained will suffice for the treatment of 500 kilos of true skins, if it is intended to tan with 3% of  $Fe_2O_3$  reckoned on the weight of the true skins employed. The solution is made up in the manner described in Example 1 with a sodium carbonate solution of 10% contents to an approximate pH value of 2, and the tanning then is effected in a corresponding manner. The subsequent second tanning with chrome tanning agents here also will be effected in the manner indicated in Example 1.

If desired, the subsequent second tanning with the chrome tanning agents or the like may also be effected without previous neutralization of the leather preliminarily tanned with iron compounds.

(3) Instead of the subsequent second tanning being performed by means of chrome compounds, aluminium compounds may also be employed for this purpose. In this case the leathers, after having completed the iron tanning process described, are fulled with 50 kilos of alum or with the corresponding quantity of aluminium sulphate and 100% of water. By gradual addition of a 10% solution of sodium carbonate, the basicity of the solution is gradually raised until the point of flocculent separation of the aluminium is nearly attained. After fulling the skins for 50 1 to 1½ hours, the second stage of the tanning process will be completed. The leathers are then washed, neutralized if necessary, greased and dressed in accordance with customary methods. The leathers treated with alum are of a very nice light colour and are distinguished by an excellent feel or touch and very good filling or body.

Instead of employing chrome shavings, parings or skins or the like, any other albuminoid substances may be used as starting materials for

preparing the tanning liquor for the first stage of the process, such as shavings of vegetably tanned leather, glue casein, waste of artificial albuminoid masses, horn, hairs, for instance calf's hairs, and decomposition products of such substances. A contents of tanning substances of the shavings or other leather waste does not adversely influence the process, but also is not decisive for its success.

Instead of nitric acid or potassium chlorate other oxidizing means, such as nitric oxides, free chlorine, potassium permanganate and the like may be used for the preparation of the ferro-albuminoid tanning agent.

Having now particularly described and ascertained the nature of my said invention, I declare that what I claim is:

1. A process of tanning hides, consisting in the hides first are tanned with a solution obtained by the treatment of albuminoid substances with acids and oxidizing means in the presence of iron salts, whereupon they are tanned a second time with other mineral tanning agents.

2. A process of tanning hides, consisting in the hides first are tanned with a solution obtained by the treatment of albuminoid substances with acids and oxidizing means in the presence of iron salts, whereupon they are tanned a second time with chrome tanning agents.

3. A process of tanning hides, consisting in the hides first are tanned with a solution obtained by the treatment of albuminoid substances with acids and oxidizing means in the presence of iron salts, whereupon they are tanned a second time with aluminium tanning agents.

4. A process of tanning hides, consisting in the hides first are tanned with a solution obtained by the treatment of albuminoid substances with acids and nitrogen-oxygen compounds in the presence of iron salts, whereupon they are tanned a second time with other mineral tanning agents.

5. A process of tanning hides, consisting in the hides first are tanned with a solution obtained by the treatment of albuminoid substances with nitric acid in the presence of iron salts, whereupon they are tanned a second time with other mineral tanning agents.

6. A process of tanning hides, consisting in the hides first are tanned with a solution obtained by the treatment of albuminoid substances with acids and a nitric oxide in the presence of iron salts, whereupon they are tanned a second time with other mineral tanning agents.

7. A process of tanning hides, consisting in the hides first are tanned with a solution obtained by the treatment of albuminoid substances with acids and chlorates in the presence of iron salts, whereupon they are tanned a second time with other mineral tanning agents.

MAX BERGMANN. 135